

Jan. 10, 1956

J. J. BECK

2,729,935

METHOD OF INCREASING THE STRENGTH OF A SPROCKET CHAIN

Filed Nov. 24, 1950

2 Sheets-Sheet 1



FIG. 1.



FIG. 2.



JOSEPH J. BECK  
INVENTOR.

BY George A. Evans  
ATTORNEY

Jan. 10, 1956

J. J. BECK

2,729,935

METHOD OF INCREASING THE STRENGTH OF A SPROCKET CHAIN

Filed Nov. 24, 1950

2 Sheets-Sheet 2

FIG. 7.



JOSEPH J. BECK  
INVENTOR.

BY *George A. Evans*  
ATTORNEY

1

2,729,935

## METHOD OF INCREASING THE STRENGTH OF A SPROCKET CHAIN

Joseph J. Beck, Milwaukee, Wis., assignor to Chain Belt Company, Milwaukee, Wis., a corporation of Wisconsin

Application November 24, 1950, Serial No. 197,297

6 Claims. (Cl. 59—8)

This invention relates to improvement in the manufacture and construction of chain of the type having curled sections at the ends of the links, the links being connected by pins extending through the curled sections thereby forming a series of hinged joints. An example of such chain is shown in U. S. Patent No. 1,966,659 to Wynne et al., and the present invention will be described in connection with chains of the type shown in the Wynne et al. patent.

It has heretofore been possible to produce chains of satisfactory strength for normal applications if the steel from which they are made is heat treated after forming to harden the links and to remove residual stresses created in the curled portions. When the chains are formed from what is commonly designated "stainless" steel of a type which it is not feasible to heat treat after forming, i. e., on account of its not responding to heat treatment, the yield strength is materially reduced because of the tendency of the curled portions to uncurl when a load is applied on the chain. This is partly caused by the application of the load on the pitch line of the chain below the plane of the link, producing a moment tending to straighten out the curled portions. But the condition is exaggerated by the retention of stresses, due to the curling operation, which are nearly up to the yield point of the material. When such a chain is placed in tension, the stresses are cumulative resulting in yielding of the chain at a low work load.

The present invention provides a method whereby the links when formed and assembled will have residual stresses in the curled portions which will help to carry the load rather than add to the load, thereby increasing the working load capacity of the chain.

The invention has utility not only in connection with austenitic steels which are not readily hardened by heat treatment, but also when applied to other metals which respond to cold working, it provides a procedure which may be used instead of heat treatment.

In the accompanying drawings, which illustrate one of the methods of practicing the invention and producing the improved chain:

Fig. 1 is an exploded, perspective view of two chain links of the type with which this invention is concerned;

Fig. 2 illustrates a link of the type shown in Fig. 1 as it is held in a die to over-curl the central knuckle at one end of the link;

Figs. 3, 4 and 5 illustrate successive changes in link contour as a result of the next forming operation;

Fig. 6 is an enlarged side elevation of the curled portion illustrating the changes in contour as a result of the working operations; and

Fig. 7 is a graph showing the stress-strain relationship of links produced by the present method compared with those made in a conventional manner.

Referring to Fig. 1 of the drawings, each of the links 11, which are formed from flat plates of metal, has a central curled portion 12 at one end and spaced curled portions 13 at the other end. The curled portions 13

2

are spaced apart a distance corresponding to the width of the central curl 12 and have cylindrical apertures of the same diameter as the aperture in the central curl so that a series of such links may be assembled end-to-end, 5 with the holes in the overlapping, interfitting curled portions aligned. By inserting a connecting pin 13' through each set of aligned curled portions, an endless chain is formed having hinged, articulating joints. The knuckles ride in grooves in the sprockets, as illustrated in the 10 Wynne et al. patent, and thus power can be transmitted to the chain to enable it to convey articles such as bottles, packages, etc.

Experience has demonstrated that when a chain of the type described above is overloaded, the central curled 15 portions 12 are the first to yield, and yielding manifests itself by the portion designated 18 lifting and tending to bend back on itself, which action will hereafter be referred to as uncurling. The result is an increase in the pitch, i. e., the distance between centers of the joints at the ends of each link, and such increase destroys proper action of the chain over the sprockets.

The present invention provides a method whereby residual compressive stresses instead of tension stresses are created in the inside surface of the curled portion, which stresses resist the above described uncurling and greatly increase the yield strength.

From a practical standpoint, only the central curled portion 12 requires strengthening and the operations hereafter set forth will be described only in connection 30 with that portion. Should it be necessary however to strengthen the curled portions 13, it will be appreciated that the same technique may be applied to do so.

In Fig. 2, the link formed in the conventional manner is placed in a fixed die member 14 which confines the 35 spaced knuckles 13 and the flat central portion 15 of the link so that these portions are not affected by the forming operation illustrated in this figure. Relief is provided at 16 in the die 14 so that when the movable die 17 comes down on the back of the central curl 12, 40 this portion of the link will be further curled or over-curved by shortening the pitch and increasing the distance from the center of the curl to the plane of the link.

The shape of the link after the above operation is 45 illustrated in Fig. 3; the radius of curvature in the region designated 18 has been increased so that with the bottom portions 19 and 20 of the curled sections 12 and 13 respectively resting on horizontally aligned surfaces of the die 21, the flat portion 15 of the link slopes downwardly from the right to left as shown in said figure. 50 The link is then brought to final shape by the die action illustrated in Fig. 4.

In Fig. 4, the movable die member 22 is illustrated 55 engaging the flat central portion 15 of the link, while the opposite side of said portion as well as the two curled sections are resting on the die 21. The portion 18 of the curled section 12 is sprung upward just enough so that when the die 22 is retracted, as illustrated in Fig. 5, the correct final shape will result on account of "spring-back" of the metal.

60 The links are then assembled to make up the chain by inserting the pins 13' through the overlapping or interfitting curled sections as previously described.

While the method has been described in connection 65 with links which were previously formed in a conventional manner, in order to illustrate more fully how the operations are performed, the step illustrated in Fig. 2 can be eliminated by initially curling the section 12 so that it assumes a shape similar to that shown in Fig. 3. In other words this step can be performed simultaneously 70 while the curled sections 13 are being curled to their correct final shape. In either event, the pitch of the link at the end of the operation is less than the ultimate de-

sired, and the curled portion is then uncurled to produce the correct pitch.

By the same token, other procedures from that described may be followed to extend the pitch to the correct degree, thereby creating stresses which resist the loads which the chain must carry. For instance, individual links may be elongated by inserting pins through the curled portions and then pulling these pins apart so that the metal of the link is stretched beyond its elastic limit and beyond the final pitch required. When the pressure is released, the curled or eye portion 12 springs back partially to produce the proper pitch. This operation does not affect the curled portion 13 for the reason heretofore mentioned that the portion 12 is the first to yield under conditions of overload.

Still another procedure is to assemble a strand of links after they are each shaped to form similar to that shown in Fig. 3 and then to grip the knuckles at the ends of the strand and pull the entire strand so that the individual links are stretched to the correct pitch. While there is some danger in the latter procedure if the links are non-uniform in physical characteristics that the individual links will be unevenly elongated, if the manufacture of the individual links is carefully performed, and uniform material is employed, remarkable pitch accuracy is obtained by this method, with resulting economy in manufacture.

The effect of the uncurling operation is illustrated in Fig. 6, wherein the full lines represent the position of the curled portion 12 of the link at the conclusion of the uncurling operation and the dotted lines the position and shape of this portion prior to its being uncurled. Residual compressive stresses have been imposed on the inside fibers of the curl at 23 and residual tension stresses on the opposite outside fibers. The center of the curl 12 has now been moved so as to form the correct pitch for the link.

In all three procedures, the stresses which are created are retained in the links when they are placed in service. Such residual stresses, i. e. stresses present when no load is applied, act in a compressive manner circumferentially on the inside of the curled portion as a result of the uncurling operation, instead of in a tensile manner, as they formerly did.

The increase in strength of the chain resulting from the present invention is illustrated by the graph shown in Fig. 7. In each test the ends of a strand of thirteen links of chain were held in fixtures and the chains were pulled apart on a tensile testing machine. Each curve represents an average of two or more tests. The load in pounds is plotted against elongation in inches.

The chain test illustrated by curve A involved a strand of standard 18-8 (18% chrome-8% nickel) stainless steel chain having one and one-half inch pitch formed in the manner employed prior to the present invention. At slightly over 200 pounds pull, A' on the graph, elongation discontinued being a straight line function of load, indicating the yield point of the chain.

The links used in the other tests, hereafter described, were made from the same material, same gauge of metal, and in every respect were as similar as possible.

Curve B represents the stress-strain relationship of a strand of chain, the individual links of which were formed by following the operation described in detail in the first part of this description, using the dies illustrated in Figs. 2-5. The yield point was increased from 215 pounds to 625 pounds, or roughly 300%.

Curve C shows an ultimate strength of 1035 pounds was obtained when the links were initially formed to the shape illustrated by Fig. 3, but instead of being subsequently formed by dies as illustrated in Figs. 4 and 5, the ends were gripped and then pulled away from each other to produce the correct chain length.

The yield point D' was obtained on curve D after the entire assembled strand of individual, underpitch links

was stretched to increase the pitch of the links to the correct dimension, the initial strand in this case having 80 links when it was stretched, sections of thirteen links thereof being taken at random for test purposes. The yield point of 950 pounds represented an increase of approximately 450% over that of standard chain illustrated in curve A.

It is essential that after the uncurling operation the pitch be as accurate as possible to the ultimate desired.

10 Any extension of the pitch beyond this will render imperfect the action of the chain over the sprockets, the teeth of which are designed in accordance with the pitch designation of the chain.

The invention having been described, what is claimed is:

15 1. The method of increasing the yield strength of a sprocket chain link having a curled joint portion at one end of the link which comprises curling said portion so that the pitch of the link is less than the ultimate desired and then uncurling said portion to increase the pitch to the desired length, said last mentioned step imparting residual compressive stresses on the inside surface of the curled portion in the area where the curled portion joins the rest of the link which are retained in the link when it is placed in service.

20 2. The method of increasing the yield strength of a chain having an intermediate curled portion at one end of each link connected in hinge fashion with spaced curled sections of an adjoining link, which method comprises overcurling the said intermediate curled portions of each link and then uncurling said portions to bring the links to the correct length and impart residual compressive stresses on the inside surfaces of said portions where they join the rest of the link.

25 3. The method of producing a chain link in a chain having joints at each end of the link, one end having a curled portion for receiving a pin hingedly connecting it with an adjoining link which comprises curling said end portion so that the pitch of the link measured by the distance between the center of the curled portion and the center of the joint at the other end of the link is less than the ultimate desired; then uncurling said end portion and allowing it to spring-back to increase the pitch the required amount, the spring-back from the uncurling operation setting up residual compressive stresses on the inside of the curled portion and increasing the yield strength of the link, and finally assembling the link in the chain with the compressive stresses still retained in the curled end portion.

30 4. The method of producing sprocket chain having links with interconnected hinged joints, each of said joints having a central curled portion connected by a pin with spaced, overlapping joint sections on an adjoining link, which method comprises curling the central curled portion of each link so that the center thereof is closer than that desired to the joint at the other end of the link, and then after connecting a plurality of such links in a strand, pulling the ends of the strand apart to bring the individual links after spring-back to the correct length, thereby setting up residual compressive stresses on the inside surfaces of the central curled portions.

35 5. The method of producing a chain link having a substantially flat central portion and curled end portions for connection with adjoining links, one curled end portion forming the intermediate section of a hinge joint with the curled sections of an adjoining link, which method comprises curling said intermediate end portion so that the pitch of the link measured by the distance between the centers of the curled portions at each end of the link is less than that desired and the center of the intermediate

40 curled portion is further from the plane of the flat central portion of the link than the center of the curled portion at the other end of the link, and then uncurling said intermediate portion to increase the pitch the required amount and align the centers of the curled portions with respect to said plane, the uncurling operation setting up residual

compressive stresses on the inside of said intermediate curled portion and increasing the yield strength of the link.

6. The method of producing a chain link having a substantially flat central section and curled end portions for connection with adjoining links, one curled end portion forming the intermediate section of a hinge joint with the curled sections of an adjoining link, which method comprises curling said intermediate end portion so that the center thereof is further from the plane of the flat central section than the centers of the curled portions at the other end of the link and then uncurling said intermediate end

5

10

portion to align the centers with respect to plane of the link, the uncurling operation setting up residual compressive stresses on the inside of said intermediate curled portion and increasing the yield strength of the link.

## References Cited in the file of this patent

## UNITED STATES PATENTS

1,966,659 Wynne \_\_\_\_\_ July 17, 1934  
2,517,497 Lauenstein \_\_\_\_\_ Aug. 1, 1950